

## UNITED STATES PATENT OFFICE

FRANK L. FROST, JR., OF EAST CLEVELAND, OHIO, ASSIGNOR TO THE GRASSELLI CHEMICAL COMPANY, OF CLEVELAND, OHIO, A CORPORATION OF DELAWARE

## TRI-SODIUM PHOSPHATE HYDRATE-SOAP COMPOSITIONS

No Drawing.

Application filed March 26, 1931. Serial No. 525,613.

Tri-sodium phosphate is usually sold as its dodecahydrate, in which form it is, however, very susceptible to caking into hard, solid lumps, which make the product very difficult to handle, particularly in the retail trade.

My invention comprises a new composition consisting of tri-sodium phosphate hydrate crystals containing a small amount of a soap as an integral constituent of the crystal and of processes of producing this composition.

I have found that when a saturated tri-sodium phosphate solution containing a small amount of a fatty or resinous acid soap is allowed to crystallize, the soap will not remain in the mother liquor, but crystallizes out with the tri-sodium phosphate and becomes an integral part of the crystals.

The appearance of the new crystals is quite different from that of straight tri-sodium phosphate dodecahydrate. While both products crystallize in the form of hexagonal prisms, the soap containing crystals have a satin like sheen or luster by which they are easily distinguished from the straight tri-sodium phosphate crystals. The main difference between the two products is, however, besides chemical composition, in their behavior towards atmospheric changes. When ordinary tri-sodium phosphate dodecahydrate is exposed to a dry or a hot atmosphere it loses part of its water of crystallization and under moist conditions takes this water up again with formation of new, small crystals which cement together the larger original individual crystals; tri-sodium phosphate crystals which contain a small amount of soap as an integral constituent lose similarly water under drying conditions, but when this water is again taken up no cementing of the larger crystals into solid lumps by formation of small intermediate crystals seems to take place, and an over-dried, soap containing tri-sodium phosphate hydrate can be kept for weeks in a moist atmosphere of, for instance, 90% saturation without substantial caking.

The amount of soap necessary to produce my novel composition does not in any way interfere with the crystallization of the prod-

uct. On the contrary, under similar conditions, the soap containing tri-sodium phosphate will develop into larger and better formed individual crystals than a straight tri-sodium phosphate will do.

The soap necessary to produce my novel composition is added preferably as an aqueous solution to the tri-sodium phosphate liquor before or after concentration and before crystallization. Another convenient method is to add resin acid or fatty acid to the phosphoric acid before neutralization, and then produce the crystals by concentration and cooling of the neutralized acid.

The amount of soap which can be made to crystallize out with tri-sodium phosphate hydrate is not very critical, and crystals with a satin like sheen are already obtained when the product contains around  $\frac{1}{10}$  % of the soap. For practical purposes amounts of less than 1% soap are preferred, and about 0.3% oleic acid soap is an amount which produces a beautiful substantially non-caking crystal. Other soaps, such as stearates, palmitates and resinates produce quite similar looking products. The soap seems to be homogeneously distributed through the crystals and forms an integral part thereof.

Instead of allowing the tri-sodium phosphate soap composition to crystallize from a concentrated solution and separating the crystals from the mother liquor, it is also possible to spray such a solution and thereby obtain evaporation of water and cooling to produce the same composition of matter.

The composition of crystals is not necessarily exactly that of dodecahydrate. As is well known in the art the water content of tri-sodium phosphate polyhydrates, that is to say those which contain more than one molecule of water of crystallization, depends upon atmospheric conditions, and in the case of the dodecahydrate may vary a few percent above or below the value for 12 mols of crystal water. The same is true with my novel soap containing tri-sodium phosphate crystals, which can contain more or less water of crystallization than corresponds to the dodecahydrate without losing their substantially non-caking properties.

I claim:

1. The process of producing a tri-sodium phosphate hydrate soap composition which comprises preparing a concentrated aqueous solution containing tri-sodium phosphate and a small amount of a soap, and inducing crystallization of the tri-sodium phosphate hydrate-soap composition in said solution.
2. The process of producing a tri-sodium phosphate hydrate-soap composition which comprises preparing a concentrated aqueous solution containing tri-sodium phosphate and less than 1% of a fatty acid soap, inducing formation of tri-sodium phosphate hydrate-soap crystals therein and separating the crystals from the mother liquor.
3. A co-crystallized tri-sodium phosphate hydrate-soap composition, the crystals of which have a satin like sheen or luster.
4. A co-crystallized tri-sodium phosphate hydrate-soap composition in which the soap is a constituent part of the individual crystals, the crystals having a satin like sheen or luster.
5. A co-crystallized tri-sodium phosphate hydrate-soap composition in which the soap is distributed throughout the body of the individual crystals, the crystals having a satin like sheen or luster.
6. A co-crystallized tri-sodium phosphate hydrate-fatty acid soap composition in which the soap is a constituent part of the individual crystals in an amount of not more than 1%, the crystals having a satin like sheen or luster.
7. A co-crystallized tri-sodium phosphate dodecahydrate-soap composition in which about 0.3% of sodium oleate is a constituent part of the individual crystals, the crystals having a satin like sheen or luster.
8. A co-crystallized tri-sodium phosphate dodecahydrate-soap composition in which about 0.3% of stearic acid soap is a constituent part of the individual crystals, the crystals having a satin like sheen or luster.

In testimony whereof, I affix my signature.

FRANK L. FROST, JR.